# EUROPEAN PATENT SPECIFICATION

(11) **EP 1 729 971 B1**
(45) Date of publication and mention of the grant of the patent: **23.07.2008**
(21) Application number: 05729450.6
(22) Date of filing: 22.03.2005
(51) Int. Cl.: B41M 5/00, B41M 5/52

(54) **INK RECEIVING MATERIAL AND METHOD FOR ITS' PREPARATION**
TINTENAUFNAHMEMATERIAL UND VERFAHREN ZUR HERSTELLUNG
MATÉRIAU RÉCEPTEUR D'ENCRE ET PROCÉDÉ POUR SA FABRICATION

(30) Priority: 27.03.2004 GB 0406981
(43) Date of publication of application: 13.12.2006
(73) Proprietor: Eastman Kodak Company, Rochester, New York 14650-2201 (US)
(72) Inventor: NEWINGTON, Ian Martin, Buckinghamshire HP13 6JR (GB); HIGGINS, John Martin, Middlesex HA5 2EZ (GB); REIGNIER, Stephanie, Marie, 75020 Paris (FR)
(74) Representative: Haile, Helen Cynthia
(86) International application number: PCT/GB2005/001058
(87) International publication number: WO 2005/095113

(56) References cited:
- EP-A- 1 266 764
- EP-A- 1 364 804
- WO-A-97/27240
- WO-A-97/37745
- US-A- 5 189 070
- US-A- 5 817 704

## Description

### FIELD OF THE INVENTION

The present invention relates to inkjet receivers and to a method of making inkjet receivers. More particularly, the invention is concerned with improved ink-receiving layers having rapid ink uptake and large capacity and to methods of making such ink-receiving layers in inkjet receivers. More specifically, the present invention relates to the use of emulsions to generate porous inkjet receivers.

### BACKGROUND OF THE INVENTION

Inkjet receivers are generally classified in one of two categories according to whether the principal component material forms a layer that is "porous" or "non-porous" in nature. Many commercial photo-quality porous receivers are made using a relatively low level of a polymeric binder to lightly bind inorganic particles together to create a network of interstitial pores which absorb ink by capillary action. These receivers can appear to dry immediately after printing. However, relatively thick layers are usually required, sometimes as much as 50 µm, to provide sufficient fluid capacity. As the component materials are relatively dense, large masses of material are needed and the layers are often prone to cracking and brittleness.

Non-porous receivers are made up of polymeric layers that are capable of absorbing relatively large amounts of ink by molecular diffusion. The main problem with this type of receiver is that the diffusion process is relatively slow and the receivers can take a considerable time before they appear dry.

A porous polymer material may be a suitable material for use in an inkjet receiver. Methods for making porous polymer materials have been known for some time, although difficulties in conveniently making porous materials with suitable physical properties without involving the use of significant quantities of volatile organic materials, particularly to create porosity, would be likely to prove disadvantageous in making inkjet receivers, especially in large scale manufacture.

However, porous polymeric foams obtained by polymerising a polymerisable monomer in a high internal phase emulsion (HIPE) are known and their use as industrial filters, as supports in synthesis and cell growth, and as absorbent materials for sanitary articles has been described.

WO-A-97/37745 describes a method of preparing a filter material for use as a bag filter, for example, by impregnating a HIPE comprising a polymerisable monomer in the continuous phase into a porous substrate, such as a felt material, and polymerising the polymerisable monomers to form a cured foam within the felt material. The filter material formed can comprise mean pore sizes of between about 1 and 100 µm. The small pore size and high degree of porosity of the material formed results in a significant reduction in the pressure drop across the filter material.

US-A-5817704 describes a HIPE-derived heterogeneous polymeric foam structure of interconnecting cells, obtained by polymerising polymerisable monomers from at least two distinct HIPEs in a mixture, for use to absorb and store liquids in sanitary articles.

WO-A-97/27240 describes a method of preparing foams from HIPEs by coating a HIPE continuously onto a continuous moving strip of relatively inert polymeric film, such as polypropylene, spooling the coated polymeric film and heat curing the HIPE on the coated, spooled film. The foam can then be unspooled and removed from the polymeric film.

EP-A-1 266 764 describes an inkjet recording medium comprising fine inorganic particles and a binder, the binder comprising an emulsion resin prepared by emulsion polymerization employing a polymer dispersing agent having a hydroxyl group.

EP-A-1 364 804 relates to a coating composition suitable for inkjet printing containing a water-insoluble emulsion polymer comprising one or more cationic monomer units and one or more vinyl ester monomer units, together with pigment and water.

US 5,189,070 describes a process for the preparation of a low density porous crosslinked polymeric material by polymerizing a water-in-oil high internal phase emulsion and carrying out the curing in multiple stages.

It is desirable to form an ink-receiving layer for an inkjet receiver which absorbs large quantities of ink rapidly. It is further desirable that the ink-receiving layer is sufficiently thin that the sharpness of the printed image is maintained. It is still further desirable that an ink-receiving layer provides good light and environmental stability for the printed image.

### PROBLEM TO BE SOLVED BY THE INVENTION

It is, therefore, an object of the invention to provide a novel method of making an ink-receiving layer for an inkjet receiver, which enables rapid uptake of ink and provides high capacity.

It is a further object of the invention to prepare such an ink-receiving layer economically and efficiently and, therefore, from the minimum of material.

### SUMMARY OF THE INVENTION

According to a first aspect of the invention there is provided a process for the preparation of an inkjet receiver having a liquid-receiving layer with a high liquid-absorption rate, said process comprising the steps in the order given:- generating an emulsion comprising a first phase having a first carrier fluid and a second phase having a second carrier fluid, said first and second carrier fluids being immiscible; coating the emulsion onto a support; carrying out a first treatment to at least one component of the first phase to form and/or maintain a skeletal structure of the at least one component of the first phase in the emulsion; and carrying out a second treatment to the second phase to substantially remove the second carrier fluid, thereby generating a large capacity porous structure defined by the skeletal structure for rapid uptake of ink.

In a second aspect of the invention, there is provided an inkjet receiver comprising a porous cross-linked polymeric liquid-receiving layer comprising a polyHIPE material obtainable by the above process, wherein the polyHIPE material is defined by a skeletal structure comprising pores of an average pore size of 0.1 µm or less.

There is also described the use of an emulsion to form a porous cross-linked polymeric liquid-receiving layer for an inkjet receiver by coating the emulsion onto a support, treating at least one phase of the emulsion to form a skeletal polymer structure and removing at least one other phase of the emulsion.

Further disclosed is the use of high shear applied to an emulsion to control the pore size of a porous cross-linked polymeric material prepared therefrom.

There is also described herein a method of printing, said method comprising the steps of providing an inkjet printer responsive to electronic data signals, loading the inkjet printer with an inkjet receiver as defined above and causing electronic data signals, corresponding to a desired image to be printed, to be sent to the inkjet printer, said inkjet printer responding by printing the image onto the inkjet receiver.

### ADVANTAGEOUS EFFECT OF THE INVENTION

The process of the present invention provides an ink-jet receiver that is capable of rapid uptake of large amounts of ink due to the large internal, open-cell capacity formed within the skeletal structure of the porous cross-linked polymer formed.

### BRIEF DESCRIPTION OF THE DRAWINGS

Fig. 1 shows a cross-sectional Scanning Electron Micrograph (SEM) of a conventional porous polymeric material obtained by heat-curing in a mold a HIPE formed by a conventional low shear process;
Fig. 2 shows a cross-sectional SEM of a porous polymeric liquid-receiving layer of an inkjet receiver prepared by heat-curing a HIPE-coated support according to the present invention.
Fig. 3 shows a graph of drop volume (picolitres) versus time (milliseconds), which illustrates the rate of absorption of a porous polymeric liquid-receiving layer of an inkjet receiver prepared by heat-curing a HIPE-coated support according to the present invention.
Fig. 4 shows a graph of drop volume (picolitres) versus time (milliseconds), which illustrates the rate of absorption of a swellable polymeric liquid-receiving layer according to Comparative Example 1.
Fig. 5 shows a graph of drop volume (picolitres) versus time (milliseconds), which compares the rate of absorption of a porous polymeric liquid-receiving layer of an inkjet receiver prepared by heat-curing a HIPE-coated support according to the present invention with two commercially available inkjet receivers.
Fig. 6 shows a cross-sectional SEM of a porous polymeric liquid-receiving layer of an ink-jet receiver prepared by heat-curing a HIPE-coated support according to the present invention, in which the HIPE is mixed at a shear rate of 2000 rpm.
Fig. 7 shows a cross-sectional SEM as in Fig. 6 but in which the HIPE is mixed at a shear rate of 4000 rpm.
Fig. 8 shows a cross-sectional SEM shows a cross-sectional SEM as in Fig. 6 but in which the HIPE is mixed at a shear rate of 6000 rpm.
Fig. 9 shows a graph of mean pore diameter (µm) versus shear rate (rpm) for porous polymeric liquid-receiving layers of inkjet receivers prepared by heat-curing a HIPE-coated support according to the present invention.
Fig. 10 shows a cross-sectional SEM of a porous polymeric liquid-receiving layer of an inkjet receiver prepared by heat-curing a HIPE-coated support according to the present invention, the HIPE containing a porogen in the continuous phase.
Fig. 11 shows a top view SEM of a porous polymeric liquid-receiving layer of an inkjet receiver prepared by heat-curing a HIPE-coated support according to the present invention, in which the polymerisation initiator precursor was azobisisobutyronitrile (AIBN).
Fig. 12 shows a top view SEM, at a magnification of 5000x, of a porous polymeric liquid-receiving layer of an inkjet receiver prepared by heat-curing a HIPE-coated support according to the present invention, in which the HIPE was coated onto the support by extrusion coating.
Fig. 13 shows a cross-sectional SEM, at a magnification of 625x, of a porous polymeric liquid-receiving layer of an ink-jet receiver prepared by heat-curing a HIPE-coated support according to the present invention, in which the HIPE was coated onto the support by extrusion coating.
Fig. 14 shows a top view SEM, at a magnification of 5000x, as in Fig. 12, in which the HIPE was coated onto the support by extrusion coating at a slow extrusion rate (7 ml/min).

### DETAILED DESCRIPTION OF THE INVENTION

The emulsion used to put the present invention into effect is preferably a biphasic emulsion, typically comprising two liquid phases, which may be two immiscible oil phases, but preferably the carrier fluid in one of the phases is a lipophilic liquid and in the other is water, such that the emulsion is a water-in-oil or an oil-in-water emulsion. One of the phases may be treated to form an integral or skeletal structure such that on removal of the other phase or of a large portion of the other phase of the emulsion, for example by removal of the carrier fluid, the integrity of the structure of the first phase in the emulsion is largely maintained, thereby forming a porous structure useful for rapid uptake of liquid.

Preferably one of the phases of the emulsion - the phase to be treated such that a skeletal structure is formed - comprises a polymerisable monomer which may be treated by initiating a polymerisation reaction to form an integral polymeric structure throughout that phase, the structure remaining largely intact on removal of the carrier fluid of the other phase. Alternatively, the phase of the emulsion to be treated such that a skeletal structure is formed may comprise a soluble polymer, which may be treated by initiating a cross-linking reaction. Suitable soluble polymers include polymers of intrinsic microporosity (PIMs) such as those described in McKeown et al (J. Chem. Soc., Chem. Commun., 2004, 230-231).

In a preferred embodiment of the invention, the emulsion used according to the present invention is a high internal phase emulsion (HIPE). A high internal phase emulsion is a term known in the art and refers to emulsions in which the internal phase is present in an amount greater than would normally be expected according to spherical close-packing before inversion of the phases occurs. For example, under normal circumstances, in an oil-in-water emulsion, when the amount of the internal phase (in this case, oil) exceeds 75.04 % by volume, the emulsion would undergo phase inversion to form a water-in-oil emulsion, or vice versa. A HIPE is an emulsion which, for some reason, when the internal phase exceeds 75.04 % does not undergo such phase inversion. Usually such HIPEs require stabilisation to prevent phase inversion. For example, the emulsion may be stabilised by incorporating a suitable surfactant into the emulsion.

According to the preferred embodiment, the continuous phase (external phase) of the HIPE preferably comprises a component, such as a polymerisable monomer, which may be treated, for example by initiating a polymerisation reaction, so that a skeletal structure is formed which substantially maintains the geometrical form of the continuous phase of the emulsion. The carrier fluid of the internal phase may then be removed to reveal a highly porous skeletal structure capable of absorbing a large amount of ink. Such a skeletal structure prepared from a HIPE shall be referred to herein as a polyHIPE structure.

A particular advantage of treating the continuous phase of a HIPE to form a skeletal structure for use as a liquid-receiving layer of an inkjet receiver, besides the advantage of having a structure with a large capacity for ink, is that the internal phase defines cavities with a high degree of interconnectivity. Particular advantages of this are that, for example, the carrier fluid of the internal phase can be rapidly removed from the structure formed by treatment of the continuous phase and that it allows the rate of fluid uptake by the remaining structure to be significantly increased.

When a HIPE is formed from an aqueous phase and an oil phase, an oil-in-water HIPE may be used in which a component in the aqueous phase is treated to form an integral structure defined by the structure of the aqueous phase in the emulsion. Preferably, however, a water-in-oil HIPE is utilised.

According to the embodiment of the invention in which a water-in-oil HIPE is utilised, a component of the oil phase, which may be the carrier fluid, is preferably a polymerisable monomer that may be treated by initiating a polymerisation reaction.

The polymerisable monomer may be any suitable monomer capable of forming a polymer under reaction conditions that can be carried out in an emulsion. Suitable monomers for use according to the present embodiment include monomers having a polymerisable vinyl group such as: monoalkenyl arene monomers, for example α-methylstyrene, chloromethylstyrene, vinylethylbenzene and vinyl toluene; acrylate and methacrylate esters, for example 2-ethylhexyl acrylate, n-butyl acrylate, isobutyl acrylate, t-butyl acrylate, hexyl acrylate, n-butyl methacrylate, lauryl methacrylate, and isodecyl methacrylate; conjugated diolefins such as butadiene, isoprene, and piperylene; allenes, for example allene, methyl allene and chloroallene; olefin halides, for example vinyl chloride, vinyl fluoride; and polyfluoroolefins. A preferred polymerisable monomer according to the present invention is styrene. In any case, it is preferable that the polymerisable monomer according to the present embodiment has a low solubility in water, and more preferably is insoluble in water.

Optionally, the oil phase may comprise two or more polymerisable monomers, which monomers may, for example, be selected from the above list of monomers, so as to form a copolymer therefrom following the polymerisation reaction.

Preferably, in order to confer a degree of rigidity into the skeletal structure formed a cross-linker may be incorporated into the oil phase. Suitable cross-linking agents may be any multi-functional unsaturated monomer capable of reacting with the polymerisable monomer. Such cross-linking agents contain at least two functional groups, which functional groups may be selected from, for example, vinyl groups, acrylate groups and methacrylate groups. The cross-linking monomers may include, for example, di-functional unsaturated cross-linking monomers such as divinylbenzene, diethylene glycol dimethacrylate, 1,4-butanediol dimethacrylate and allyl methacrylate and tri-, tetra- and penta-functional unsaturated cross-linking monomers, such as trimethylolpropane trimethacrylate, pentaerythritol tetramethacrylate, trimethylolpropane triacrylate and pentaerythritol tetraacrylate, glucose pentaacrylate, glucose diethylmercaptal pentaacrylate, and sorbitan triacrylate; and poly-functional unsaturated cross-linking monomers such as polyacrylates (e.g. sucrose per(meth)acrylate and cellulose (meth)acrylate). The preferred cross-linkers are divinylbenzene and 1,4-butanediol dimethacrylate, preferably divinylbenzene.

In order to achieve an acceptable balance between the degree of rigidity of the integral structure and the flexibility of the inkjet receiver formed, so that both the integral structure and the inkjet receiver formed are suitably resilient, the relative amount of cross-linker to polymerisable monomer is preferably in the range of from 0.5 wt% to 70 wt%, more preferably from 2 wt% to 40 wt% and still more preferably from 5 wt% to 20 wt%.

Specific properties, including rate of polymerisation, flexibility, bulk, rigidity and brittleness may be controlled by varying the relative amounts of polymerisable monomers and of cross-linking agent and may depend on the specific identity of these components.

According to the present embodiment, in which a water-in-oil HIPE is utilised and the oil phase comprises a polymerisable monomer, the first treatment carried out to the at least one component (the polymerisable monomer), so that a skeletal structure is formed, is the initiation of a polymerisation reaction.

The initiation of the polymerisation reaction may be by simply heating the emulsion comprising a polymerisable monomer composition, by irradiation with UV or other electromagnetic irradiation, but preferably by heating the emulsion to form a polymerisation initiator species, e.g. a radical initiator, from an initiator precursor present in the emulsion.

Examples of suitable initiator precursors include oil-soluble initiator precursors and water-soluble initiator precursors. Suitable water-soluble initiator precursors include, for example, persulfates such as potassium or sodium persulfate, and redox coupler initiator systems such as ammonium persulfate together with sodium metabisulfite. Suitable oil-soluble initiator precursors include, for example, azo compounds such as azobisisobutyronitrile (AIBN); peroxides such as benzoyl peroxide, methyl ethyl ketone peroxide, alkylperoxycarbonates such as di-2-ethylhexylperoxydicarbonate and di(sec-butyl)peroxydicarbonate and alkyl peroxycarboxylates such as t-butylperoxyisobutyrate, 2,5-dimethyl-2,5-bis(2,3-ethylhexanoylperoxy)hexane, and t-butyl peroctoate.

Preferable alkylperoxycarbonates are branched at the 1-position and preferable alkylperoxycarboxylates are branched at the α-position and/or 1-position. Examples of branched alkylperoxycarbonates and alkylperoxycarboxylates are described in WO-A-9737745 (page 8, line 14 to page 9, line 5).

The preferred initiator precursor according to the present invention is one or more of potassium persulfate, AIBN and a redox coupler initiator system comprising, for example, ammonium persulfate and sodium metabisulfite. The initiator precursor may form part of the oil phase (e.g. AIBN) or the aqueous phase (e.g. potassium persulfate or an aqueous redox coupling system) or both (e.g. AIBN in the oil phase and potassium persulfate in the aqueous phase), but preferably the initiator precursor forms part of the aqueous phase.

Without being bound by theory, it is believed that by initiating the polymerisation reaction using an initiator in the aqueous phase, the polymer is first formed at the boundary between the oil and aqueous phases leading to better maintenance of the integral structure of the oil phase on completion of the polymerisation reaction, as compared with an initiator in the oil phase which may result in some distortion of the integral structure of the emulsion on completion of the reaction.

Nevertheless, it may be that the presence of an initiator precursor in both the oil phase and the aqueous phase may be preferred in order to ensure more rapid completion of the polymerisation reaction, which may be of particular benefit from a large scale manufacturing point of view.

The amount of the initiator precursor present and the temperature applied determines the average chain length in linear polymer systems: the more initiator, the more radicals are generated at any one time. Preferably, the initiator precursor is present in an amount of from 0.5 to 10 wt%, more preferably 1 to 7 wt% and most preferably 3 to 5 wt%, based on the amount of polymerisable monomer present.

The temperature applied during the polymerisation step (or curing step) is preferably in the range 40-120°C, more preferably 50-90°C and most preferably 60-80°C. The time for the polymerisation step is typically inversely related to the temperature applied. For example, in a preferred embodiment, the polymerisation stage involves heating to 65-70°C for a period of 4-6 hours. After the polymerisation step, the polyHIPE material formed is preferably treated by drying, in order to remove water by evaporation. Preferably the polyHIPE is dried at 65-70°C for 2-4 hours.

As mentioned above, a HIPE is usually stabilised by a surfactant. For water-in-oil emulsions, it is necessary for the surfactant to be soluble in the oil phase and suitable such surfactants may be determined according to the hydrophilic-lipophilic balance (HLB value) of a surfactant. Typically, suitable surfactants have very limited solubility in the internal phase (e.g. the aqueous phase of a water-in-oil emulsion) in order that they can adequately stabilise the HIPE and prevent phase inversion occurring spontaneously. Preferably, the surfactant has an HLB value in the range of from 2 to 6 and preferably is about 4.

The surfactant may be non-ionic, cationic, anionic or amphoteric, provided that the surfactant or combination of surfactants is effective to form a stable HIPE. Preferred types of surfactants that can be used to stabilise water-in-oil HIPEs include sorbitan fatty acid esters, polyglycerol fatty acid esters, polyoxyethylene fatty acids and esters. Examples of sorbitan fatty acids esters include sorbitan monolaurate (available as SPAN^{®} 20), sorbitan monooleate (SPAN^{®} 80) and combinations of sorbitan monoleate (SPAN^{®} 80) with sorbitan trioleate (SPAN^{®} 85). One such surfactant combination of sorbitan fatty acid esters is the combination of sorbitan monooleate and sorbitan trioleate in a weight ratio greater than or equal to 3:1, more preferably 4:1. Other suitable surfactants are "TRIODAN^{®} 20", which is a polyglycerol ester available from Grindsted^{®}, and "EMSORB^{™} 252", which is a sorbitan sesquioleate available from Henkel^{®}.

Preferred surfactants according to the preferred embodiment of the invention include, for example, sorbitan monooleate and glycerol monooleate. Sorbitan monooleate is a particularly preferred surfactant because it can also act as an ozone scavenger, which has the benefit that in the resulting inkjet receiver the surfactant can help postpone the onset of any ozone-induced fade.

The surfactant may be present in the emulsion in an amount of from 1 to 50 wt%, preferably 5 to 40 wt%, more preferably 15 to 40 wt%, still more preferably 20 to 35 wt% and most preferably 25 to 33 wt%, based on the amount of polymerisable monomer present. Where sorbitan fatty acid esters are used as a component of the surfactant, the sorbitan fatty acid ester surfactants are preferably present in an amount of from 2 to 36 wt%, more preferably from 5 to 25 wt%.

Preferably, according to the present embodiment of the invention in which a water-in-oil HIPE is utilised, the oil phase comprises a polymerisable monomer, a surfactant and optionally a cross-linker. The carrier fluid may be the polymerisable monomer or a mixture of the components or may be an additional solvent, but preferably comprises the polymerisable monomer. The aqueous phase comprises water as the carrier fluid and optionally an electrolyte for additional stabilisation of the emulsion.

Suitable electrolytes include inorganic salts (monovalent, divalent, trivalent or mixtures thereof), for example, alkali metal salts, alkaline earth metal salts and heavy metal salts, which may be halides, sulfates, carbonates, phosphates and mixtures thereof. Preferably, a suitable electrolyte comprises one or more of sodium chloride, sodium sulfate, potassium chloride, potassium sulfate, lithium chloride, magnesium chloride, calcium chloride, magnesium sulfate and aluminium chloride. Preferably, the electrolyte is calcium chloride.

Additional components may be added to the second phase according to the present invention to provide improved properties to the resulting liquid-receiving layer of the inkjet receiver. Such additional components may be, for example, swellable polymers or other materials capable of absorbing ink and/or protecting the ink from environmental factors. By incorporating such additional components into the second phase of the emulsion, these components may be evenly coated onto the surface of the skeletal structure on removal of the second carrier fluid.

Where the second phase is an aqueous phase, such as in the preferred embodiment of the invention utilising a water-in-oil HIPE, additional components that may be included in the aqueous phase to improve the properties of the resulting liquid-receiving layer of the inkjet receiver include, for example, polyvinyl alcohol (PVA) or other aqueous soluble swellable polymer material, so that on removal of the second carrier fluid (water), the PVA or other polymer material forms a thin coating on the internal surface of the resultant skeletal polymer structure. Such a coating of PVA or other swellable polymer material may provide a protective environment within the porous liquid-receiving layer for ink rapidly absorbed into the structure, especially when the liquid-receiving layer is the ink-receiving layer. Similarly, a coating of a mordant material may be formed by incorporating a mordant into the second phase. Examples of useful mordants, for stabilising absorbed ink and improving image density include for example, [3-(methacryloylamino)propyl] trimethylammonium chloride.

Other additional components that may be added to the second phase include, for example, stabilisers for dyes and/or pigments against degradation by, for example, light or ozone, UV absorbers, sequestering agents, surfactants and polymeric binders.

It has been found that HIPEs can be coated as a thin layer onto a support and treated to form a polyHIPE liquid-receiving layer of an inkjet receiver, especially an ink-receiving layer. PolyHIPE materials have been found to be advantageous for use as liquid-receiving layers in inkjet receivers, and especially as ink-receiving layers, because of their rapid rate of ink absorption and their high internal capacity, both of which features are highly beneficial for an ink-receiving layer material, because a large amount of ink can be absorbed rapidly allowing the inkjet receiver to appear dry almost immediately. For example, the graphs in Fig. 5 compare the rate of drying of an inkjet receiver made according to the present invention with two commercially available receivers. This prevents the smudging of images on the inkjet receiver or even partial transfer onto other surfaces, allowing the printed image to be handled without delay.

Another advantage is that due to the high internal capacity of polyHIPE liquid- or ink-receiving layers, a much thinner layer is required to absorb a certain amount of ink. The benefit of this is that less material is required to form the inkjet receiver, manufacturing is easier and the physical quality of the inkjet receiver is improved. TABLE 1 illustrates the effect of porosity on the volume of material and layer thickness sufficient to absorb 25 ml/m² of ink, the values corresponding to estimated values of various types of inkjet receivers mentioned in the comments column.

**TABLE 1:**

| Layer thickness and volume of material required to contain 25 ml/m² of ink for ink-receiving layers of a range of porosities. | | | |
|---|---|---|---|
| **Porosity (as %)** | **Volume of Material (ml m⁻²)** | **Layer Thickness (µm)** | **Comment** |
| 25% | 75.0 | 100.0 | Close-packed particulate structures |
| 30% | 58.3 | 83.3 | \| |
| 40% | 37.5 | 62.5 | ↓ |
| 50% | 25.0 | 50.0 | Typical Commercial Receiver |
| 60% | 16.7 | 41.1 | ↓ |
| 70% | 10.7 | 35.7 | |
| 80% | 6.3 | 31.3 | Poly(HIPE) |
| 90% | 2.8 | 27.8 | ↓ |

The porosity of the material forming the liquid-receiving layer according to the present invention depends upon several factors. In particular, the porosity depends upon the relative amounts of the first and second phases of the emulsion from which the liquid-receiving skeletal structure is formed, since the pores are defined by the second phase of the emulsion, the carrier fluid of which is removed during the process of forming the liquid-receiving layer. For example, for a water-in-oil HIPE to result in a polyHIPE material with a porosity of 80%, it is required that the HIPE comprises 20% oil phase and 80% aqueous phase. Therefore, by increasing the relative amount of the second phase in the emulsion, the porosity of the resultant liquid-receiving layer may also be increased.

It further depends upon the quantity of addenda included in the second phase.

The porosity of the skeletal structure formed may be further increased by incorporating a porogen into the first phase of the emulsion (e.g. the oil phase of a water-in-oil HIPE according to the preferred embodiment). The degree of porosity may be controlled according to the amount and the identity of the one or more porogens used. Examples of suitable porogens include any organic solvent soluble in the oil phase but not substantially water-soluble. The precise identity may depend upon the polymerisable monomer used, but examples include hexane, cyclohexane, heptane and, preferably, toluene.

Preferably the polyHIPE formed according to the preferred embodiment of the present invention has a porosity of at least 26%, such as within the range 30-95%, and more preferably in the range 40-90%. In a preferred example, the polyHIPE formed may have a porosity in the range 60-85%.

Preferably, the liquid-receiving layer described above in accordance with the present invention, is an ink-receiving layer of an inkjet receiver.

An ink-receiving layer according to the present invention, and particularly the preferred embodiment of the invention in which a water-in-oil HIPE is utilised, is preferably formed having a thickness of 200 µm or less, more preferably 100 µm or less, still more preferably 50 µm or less and most preferably in the range of from 5 µm to 45 µm, the precise thickness depending also upon the degree of porosity of the ink-receiving layer formed, the design of the inkjet receiver and the type and amount of ink to be used to print onto the inkjet receiver.

According to the present invention, the emulsion may be coated onto the support, or as part of a multi-layer structure, by any suitable coating method. For example, the emulsion may be coated by blade-, knife- or extrusion-coating techniques. One method of coating found to be effective is blade-coating. However, a preferred method of coating the emulsion may be by an extrusion-coating technique wherein the rate of extrusion may affect the resultant structure of the porous polymer material. Thus at a low rate of extrusion the structure of the resultant material may be similar to that obtained via blade-coating, whilst at a higher rate of extrusion, a modified structure may result, which still has an excellent rate of absorption and fluid capacity. For example, a relatively higher rate of extrusion may result in a modified structure - see, for example, the polyHIPE structure in Fig. 12 whilst an intermediate rate of extrusion may result in an intermediate modified structure of the porous polymer material - see, for example, the polyHIPE structure in Fig. 14.

Suitable supports for use in the present invention include any suitable support for an inkjet receiver, such as resin-coated paper, film base, acetate, polyethylene terephthalate (PET), a printing plate support such as aluminium foil, a latex-treated polyester or any other suitable support. Aluminium foil and latex-treated polyester have been found to be particularly effective supports for use in the preferred embodiment of the present invention in which a porous polymeric ink-receiving layer is formed using a water-in-oil HIPE.

Preferably, after coating of the emulsion onto the support, there is some means of preventing either of the carrier fluids from evaporating in substantial amounts before or during the step in which the first phase is treated. For example, in the case of a water-in-oil HIPE, there is some means of preventing evaporation of water, which could cause the emulsion to collapse, before or during the polymerisation step. One method of achieving this is to laminate the coated support, for example with a temporary plastic laminate material or with a sheet of glass, which can be removed after the polymerisation step.

The average pore size of the skeletal structure formed according to the present invention, especially in respect of the preferred embodiment in which a polyHIPE material is formed from a water-in-oil HIPE, is preferably up to about 10 µm diameter, more preferably up to 1 µm, still more preferably up to 0.1 µm and most preferably in a range from 10 to 90 nm, and perhaps within a range of from 20 to 80 nm, or from 25 to 60 nm.

A particular advantage of having a skeletal structure with a small pore size, especially a pore size of 0.1 µm or less, is that ink or other material to be absorbed can be absorbed much more quickly because of improved capillary action. Another important advantage is that the skeletal structure, e.g. a polyHIPE material, when used as an ink-receiving layer can appear much more glossy if the pore size is relatively small. A further advantage is that the emulsion from which the skeletal structure is formed is better dispersed and therefore has improved stability, which makes coating the emulsion onto a support easier and makes coating the emulsion in a thin layer, e.g. 100 µm or less, possible.

It has been found that the shear to which the emulsion is subjected can be used to control the pore size of the resultant skeletal structure. In particular when using a mixer, for example a Polytron^{™} high shear mixer, the shear rate can be used to control the pore size in the resultant material.

For example, in a water-in-oil HIPE according to the preferred embodiment of the invention, an increase in the shear rate of mixing applied to the emulsion prior to coating onto a support of from 2000 to 6000 rpm resulted in a substantial decrease in pore size, as can be seen from Figs. 6 to 9, without significantly affecting the overall pore volume of the resultant liquid-receiving layer.

Preferably, therefore, the process of generating an emulsion according to the present invention, comprises mixing the phases in a mixer with a high shear rate, having a shear rate of, for example, greater than 1000 rpm, preferably greater than 2000 rpm, for example, in the range from 4000 rpm to 6000 rpm, but preferably at least 6000 rpm and more preferably at least 7000 rpm.

When preparing the emulsion, especially in large quantities, it may be beneficial to mix the emulsion at a first shear rate in order to establish an adequately mixed emulsion for a first period, and then to increase the shear rate to a rate according to the porosity desired in the resultant material as discussed above for a second period, rather than maintain the higher shear rate for the entire mixing time, in order to prevent heat generated during the mixing process causing the polymerisation step to begin or to proceed to any great degree.

According to a preferred embodiment of the fourth aspect of the invention, there is provided the use of the shear rate of mixing an emulsion to control the pore size of a skeletal structure formed by treating a first phase of the emulsion to form the skeletal structure and removing a carrier fluid from a second phase. The use of the shear rate to control the pore size is particularly applicable to the formation of a porous polymer foam formed by polymerisation of a HIPE comprising a polymerisable monomer in the continuous phase (first phase). In particular, the use of a shear rate of, for example, 4000 to 6000 rpm may control the pore size of the porous polymer foam, or polyHIPE, formed to less than 5 µm. An increase in shear rate of from 2000 to 6000 rpm, for example, may result in pores being reduced in size from greater than 10 µm to less than 5 µm. The use of a shear rate of greater than 7000 may be used to control the pore size to be less than 1 µm.

The control of pore size to be relatively small, e.g. 0.1 µm or less, for example, within the range 10 to 80 nm may be beneficial in a variety of uses of such porous polymer foams. Such uses might include, for example, polymer foams as filters to remove from a fluid stream very small particles of dimensions similar to the average pore size of the polymeric foam. The ability to control the pore size to be very small, e.g. within the range 10 to 80 nm, is especially useful in forming an ink-receiving layer of an inkjet receiver.

Preferably, as mentioned above, the liquid-receiving layer is the ink-receiving layer and dyes in the ink may be retained by the material in that layer. The ink-jet receiver may comprise only a support and the above-described liquid-receiving layer as the ink-receiving layer and, optionally, a top coat.

Optionally, in a further aspect of the invention, the porous cross-linked polymeric layer described above, especially the polyHIPE materials, may form part of a multilayer structure having further layers above the porous cross-linked polymeric layer and/or below (i.e. between the porous cross-linked polymeric layer and the support). For example, the inkjet receiver may comprise an additional layer below the porous cross-linked polymeric layer to improve adhesion between that layer and the support. The receiver may also comprise a further layer above the porous cross-linked polymeric layer described above, which may be a thinner (typically, more expensive) top layer. Such a top layer preferably has a glossy appearance and may be a relatively non-porous swellable polymer layer or, preferably, also has some porous character. Such a top layer may optionally be the ink-receiving layer, the porous cross-linked polymer layer being a liquid-receiving layer capable of retaining large quantities of liquid. Examples of porous ink-receiving layers that may suitably coated onto an ink-receiving layer as described above to provide a multilayer inkjet receiver include those porous ink-receiving layers comprising inorganic particulate materials and polymeric binders described in US-A-2002/0142140, US-A-2002/0142139 and US-A-2002/0142138.

In one embodiment of a multilayer inkjet receiver comprising a porous cross-linked polymeric layer described above, especially a polyHIPE liquid-receiving layer, the receiver comprises more than one layer of the porous cross-linked polymeric material of this type, each layer having a similar, but preferably a different, porosity and pore size in a controlled manner, such that ink may permeate through the layers of the receiver. The use of shear rate as described above may effectively control the variation of pore size in successive layers of the polymeric layers of the inkjet receiver. Such a multilayer structure may still further comprise a porous or non-porous overcoat as set out above.

According to a still further aspect of the invention there is provided an inkjet receiver having an ink-receiving layer which ink-receiving layer comprises a polyHIPE material. The polyHIPE material as ink-receiving layer preferably has a thickness of 200 µm or less, more preferably 100 µm or less.

According to a still further aspect of the invention, there is provided the use of a polyHIPE material in an ink-receiving layer of an inkjet receiver. In each of these further aspects of the invention, the polyHIPE material may be prepared according to any suitable method and preferably by the method described above and may incorporate additional variants and features described.

The invention will now be described by way of example only and without limitation as to the scope of the invention in the following Examples.

### EXAMPLES

### Example 1

Styrene (9 ml) and divinylbenzene (1 ml, 55% purity) were mixed with sorbitan monooleate (3 ml) in a 500 ml wide-mouth plastic bottle and stirred with a Polytron high shear mixer at 4000 rpm under a blanket of nitrogen gas. A solution of calcium chloride (1 g) and potassium persulfate (0.4 g) in water (90 ml) that had been deoxygenated by bubbling nitrogen through it for 20 min. was then added over approximately 30 min. by peristaltic pump to the stirred monomers. During this addition, the stirrer head was raised as the volume in the bottle increased to ensure efficient mixing. After addition was complete, the mixture was stirred a further 10 min. at 5000 rpm.

The HIPE formed was coated at 100 µm thickness onto aluminium foil, which was then laminated with a flat polyester sheet and cured in the oven at 70°C for a minimum of 6 h. The polyester laminate was removed and the coating allowed to dry at 60°C for 2 h. The resultant coating was examined by Scanning Electron Microscopy, the SEM of a coating prepared according to Example 1 being shown in Fig. 2. Extremely rapid uptake of liquid was observed using the PISA device such that droplets were absorbed completely in about 30 millisec. A graph of droplet absorption as a function of time for a coating prepared according to Example 1 is shown in Fig. 3.

### Comparative Example 1

Styrene (4.5 ml), divinylbenzene (0.5 ml, 55% purity), sorbitan monooleate (1.5 ml) and initiator AIBN (0.2 g) were mixed and degassed with bubbling nitrogen for 20 min. The mixture was blade-coated onto a polyester support at a thickness of approximately 100 µm and the coating heated in a nitrogen atmosphere at 65°C for 12 h. Ink absorption measurements, made with the PISA device, on the resultant tacky coating clearly showed no ink absorption (Fig. 4) into the coating over 4 sec.

### Example 2

The effect of high shear stirring on the polymer structure was observed by preparing three coated polymer samples using the method of Example 1, except that each sample was prepared using a different shear rate. During the addition of the aqueous phase, the Polytron mixer was run at 2000, 4000 and 6000 rpm. SEM of the resultant samples clearly shows the reduction in size of the pore structure with increasing shear rate - see Fig.6 (shear rate 2000 rpm), Fig. 7 (shear rate 4000 rpm) and Fig. 8 (shear rate 6000 rpm). Fig. 9 shows a graphical relationship between shear rate and mean pore diameter.

### Example 3

Styrene (4.5 ml), divinylbenzene (0.5 ml, 55% purity) and sorbitan monooleate (3 ml) were dissolved in toluene (5 ml) and degassed with nitrogen bubbling for 20 min. This mixture was stirred at 300 rpm with a 6-bladed impeller (38 mm diameter) while a nitrogen-degassed solution of calcium chloride (1 g) and potassium persulfate (0.2 g) was added over approximately 1 h. by peristaltic pump. Stirring was continued for a further 5 min. and then a sample of the emulsion was placed in an oven at 60°C for 24 h. to cure, followed by heating under vacuum at 75°C to dry. From SEM (Fig. 10) it can be seen that not only has the typical polyHIPE structure been formed, but that the polystyrene itself is porous.

### Example 4

A polyHIPE coating was made following the method of Example 1 with the replacement of water by a 1.1 wt% solution of PVA (MW 31-50,000, 98-99% hydrolysed) in water. The intermediate HIPE was stable and was hand-coated onto aluminium foil in the same manner as Example 1, to give a highly absorbent coating after curing at 70°C for 15 h.

### Example 5

The method of Example 4 was repeated using a 2.5 wt% PVA in water solution. The HIPE was knife-coated onto aluminium foil, laminated with polyester and cured in the usual way to give a highly absorbent coating.

### Example 6

The method of Example 5 was repeated using a 5.6 wt% PVA in water solution to give a highly absorbent coating.

### Example 7

Following the method of Example 1, an aqueous solution comprising 80 ml potassium persulfate (0.4 g) and calcium chloride (1 g) in water mixed with 10 ml of 50 wt% [3-(methacryloylamino)propyl]trimethylammonium chloride in water was added to styrene (9 ml), divinylbenzene (1 ml) and sorbitan monooleate (3 ml) under nitrogen. The resultant cationic polymer-containing HIPE was hand-coated, laminated, cured and dried to give a highly absorbent coating.

### Example 8

In order to assess the effect of making a polyHIPE at low shear, and the effect of partial pre-curing of the HIPE before coating to reduce the propensity for stress-cracking of said coating, a polyHIPE coated support was prepared as follows. Styrene (4.5 ml), divinylbenzene (0.5 ml, 55% purity) and sorbitan monooleate (3 ml) were mixed in a 250 ml plastic container and stirred at 300 rpm with a 6-bladed impeller (38 mm diameter), while a nitrogen-degassed solution of calcium chloride (1 g) and potassium persulfate (0.2 g) was added over approximately 1 h. by peristaltic pump. Stirring was continued for a further 5 min. and then the resultant HIPE in the plastic container was placed in an oil bath at 60°C to cure. Samples were removed at time 0, 1.5 h. and 3 h. and coated onto glass, covered, then curing completed and the samples dried by heating under vacuum at 75°C. The sample without pre-curing collapsed completely, the sample pre-cured for 1.5 h. shrank considerably and did not produce a coherent coating, whilst that pre-cured for 3 hours showed a highly absorbent, coherent coating.

### Example 9

The method of Example 1 was followed, except that 1,4-butanediol dimethacrylate was used in place of divinylbenzene. A highly absorbent coating was produced.

### Example 10

The method of Example 1 was followed, except that glycerol monooleate was used in place of sorbitan monooleate. A highly absorbent coating was produced.

### Example 11

Styrene (9 ml) and divinylbenzene (1 ml, 55% purity) were mixed with sorbitan monooleate (3 ml) and initiator AIBN (0.4 g) in a 250 ml wide-mouth plastic bottle and stirred with a Polytron high shear mixer at 4000 rpm under a blanket of nitrogen gas. A solution of calcium chloride (1 g) in water (90 ml) that had been deoxygenated by bubbling nitrogen through it for 20 min. was then added over approximately 30 min. by peristaltic pump to the stirred monomers. During this addition, the stirrer head was raised as the volume in the bottle increased to ensure efficient mixing. After addition was complete, the mixture was stirred a further 10 min. at 5000 rpm.

The HIPE was coated at 100 µm thickness onto aluminium foil, laminated with a piece of flat polyester and cured in the oven at 70°C for a minimum of 6 h. The polyester laminate was removed and the coating allowed to dry at 60°C for a minimum of 2 h. The resultant coating was examined by Scanning Electron Microscopy (Fig. 11) and showed a slightly different polymer structure, but the coating was still very highly absorbent.

### Example 12

A polyHIPE coating was prepared using a redox coupler initiator system as follows. A solution of ammonium persulfate (0.1 g) and calcium chloride (1 g) in water (45 ml) was sparged with nitrogen gas for 20 min. Another solution of sodium metabisulfite (0.08 g) in water (45 ml) was also sparged with nitrogen for 20 min. The two solutions were mixed and addition to the monomer and surfactant mixture immediately started following the method of Example 1. Three coatings were made on a latex-coated polyester base and laminated with clean polyester sheet, then cured at different temperatures overnight: 25°C, 40°C and 50°C followed by drying at 60°C after removing the polyester laminate sheet.

All three coatings were highly absorbent, the 50°C cured sample absorbing the drop in some 40 ms, although the sample cured at 25°C was less porous as evidenced by SEM.

### Example 13

A polyHIPE coating was prepared using initiator in both aqueous and organic phases as follows. The organic phase was made up as for Example 11 and the aqueous phase as for Example 1. Following the process described in Example 1, the coating was found to be less porous with less well-defined structure but still highly absorbent.

### Example 14

A polyHIPE coating was prepared using a redox coupler initiator in the aqueous phase and AIBN in the organic phase as follows. The organic phase was prepared as in Example 11 and the aqueous phase as in Example 12. The resultant polyHIPE coating on aluminium foil was highly porous and absorbent.

### Example 15

A polyHIPE coating was prepared in which the HIPE was coated onto the support by extrusion-coating. The HIPE was prepared according to Example 1 and a syringe pump and hopper was used to extrude a thin layer onto latex-coated polyester. The coated layer was then laminated with untreated polyester and cured at 70°C for 12 h., the laminate removed and the sample dried at 60°C for a minimum of 2 h. The coating had good porosity and absorbency. Fig. 12 shows a top view SEM of such a coating at 5000x magnification and Fig. 13 shows the same coating as a cross-sectional SEM at 625x magnification. The effect of reducing the rate of extrusion (to 7 ml/min) can be seen in Fig. 14, which is a top view SEM at 5000x magnification and shows a coating that has a mixture of structures.

### Example 16

A practical assessment of the porosity of the poly(HIPE) materials was made as follows. A substantial volume of the poly(HIPE) was fully immersed in water for 5 min., carefully removed, weighed immediately and placed in a desiccator. The sample was reweighed periodically until a consistent reading was obtained, which indicated the complete removal of water from the pore system. The porosity of the sample was calculated from these data together with a knowledge of the density of water and the component materials as: $Porosity \left(%\right) = \frac{VoidVolume}{TotalVolume} \times 100$
That is, in this case: $Porosity \left(%\right) = \frac{WetVolume - DryVolume}{WetVolume} \times 100$

**TABLE2:**

| Measured porosity of various polyHIPE coatings | |
|---|---|
| **Example No.** | **Porosity** |
| 1 | 84.5 |
| 2 (4000rpm) | 84.9 |
| 2 (6000rpm) | 84.2 |
| 3 | 90.0 |

As can be seen from TABLE 2, the ink-receiving layers formed according to Example 2 at 4000 and 6000 rpm, which had substantially reduced pore dimensions as compared with the ink-receiving layer formed according to Example 1, had approximately the same degree of porosity as that formed according to Example 1. The shear rate of mixing the emulsion therefore affected the pore size, without a significant effect on the overall porosity of the ink-receiving layer formed. The ink-receiving layer formed in Example 3, however, in which a porogen was added to the oil phase of the emulsion, had a substantially greater degree of porosity as compared with that prepared according to Example 1.

## Claims

1. A process for the preparation of an inkjet receiver having a liquid-receiving layer, the process comprising the steps in the order given:-
generating an emulsion comprising a first phase having a first carrier fluid and a second phase having a second carrier fluid, the first and second carrier fluids being immiscible;
coating the emulsion onto a support;
carrying out a first treatment to at least one component of the first phase to form and/or maintain a skeletal structure of the treated at least one component of the first phase; and
carrying out a second treatment to the second phase to substantially remove the carrier fluid,
thereby generating a large capacity porous structure defined by the skeletal structure for rapid uptake of ink.

2. A process according to claim 1, wherein the emulsion is a biphasic emulsion comprising an oil phase as the first phase and an aqueous phase as the second phase.

3. A process according to either of the preceding claims, wherein the emulsion is a high internal phase emulsion.

4. A process according to any one of the preceding claims, wherein one component of the first phase is a polymerisable monomer and the first treatment is a polymerisation step for polymerising the polymerisable monomer, thereby forming the skeletal structure.

5. A process according to claim 4, wherein the polymerisation step is initiated by heating at least one initiator precursor being comprised in the aqueous phase and/or at least one initiator precursor being comprised in the oil phase.

6. A process according to claim 5, wherein the polymerisation step is initiated by heating at least one initiator precursor in the aqueous phase and wherein the initiator precursor is potassium persulfate.

7. A process according to any one of claims 4 to 6, wherein the at least one polymerisable monomer comprises one or more of styrene, α-methylstyrene, chloromethylstyrene, vinylethylbenzene, vinyltoluene, 2-ethylhexyl acrylate, n-butyl acrylate, isobutyl acrylate, t-butyl acrylate, hexyl acrylate, n-butyl methacrylate, lauryl methacrylate, isodecyl methacrylate butadiene, isoprene, piperylene, allene, methyl allene, chloroallene, vinylchloride, vinylfluoride and polyfluoroolefins.

8. A process according to any one of claims 2 to 7, wherein the oil phase further comprises at least one cross-linker monomer.

9. A process according to claim 8, wherein the cross-linker monomer is divinylbenzene.

10. A process according to any one of claims 2 to 9, wherein the emulsion further comprises a high internal phase emulsion stabilising surfactant which comprises sorbitan monooleate and/or glycerol monooleate.

11. A process according to any one of the preceding claims, wherein the first phase further comprises a porogen.

12. A process according to any one of claims 2 to 11, wherein the aqueous phase further comprises a water-soluble swellable polymer.

13. A process according to claim 12, wherein the water-soluble swellable polymer is polyvinyl alcohol.

14. A process according to any one of claims 2 to 13, wherein the emulsion is generated by mixing the oil phase and the aqueous phase in a mixer at a shear rate of greater than 2000 rpm.

15. A process according to any one of the preceding claims, wherein the skeletal structure comprises pores of an average pore size of 0.1 µm or less.

16. A process according to any one of the preceding claims, wherein the skeletal structure comprises a porous cross-linked polymeric material.

17. An inkjet receiver comprising a porous cross-linked polymeric liquid-receiving layer comprising a polyHIPE material, obtainable by the process as defined in any one of claims 1 to 16, wherein the polyHIPE material is defined by a skeletal structure comprising pores of an average pore size of 0.1 µm or less.

18. The use of a polyHIPE material in an ink-receiving layer of an inkjet receiver.

## Patentansprüche

1. Verfahren zur Herstellung eines eine Flüssigkeitsempfangsschicht umfassenden Tintenempfangselements mit den Schritten in folgender Reihenfolge:
Herstellen einer Emulsion aus einer ersten Phase mit einer ersten Trägerflüssigkeit und einer zweiten Phase mit einer zweiten Trägerflüssigkeit, wobei die erste und zweite Trägerflüssigkeit nicht mischbar sind;
Auftragen der Emulsion auf einen Träger;
Ausführen einer ersten Behandlung mindestens einer Komponente der ersten Phase zum Ausbilden und/oder Erhalten einer Skelettstruktur der behandelten, mindestens einen Komponente der ersten Phase; und
Ausführen einer zweiten Behandlung der zweiten Phase, um die Trägerflüssigkeit im Wesentlichen zu entfernen,
**dadurch** Erzeugen einer durch die Skelettstruktur definierten porösen Struktur mit großer Kapazität zur schnellen Tintenaufnahme.

2. Verfahren nach Anspruch 1, worin die Emulsion eine Bi-Phasenemulsion aus einer Ölphase als erster Phase und einer wässrigen Phase als zweiter Phase ist.

3. Verfahren nach einem der vorausgehenden Ansprüche, worin die Emulsion eine Emulsion mit hoher interner Phase ist.

4. Verfahren nach einem der vorausgehenden Ansprüche, worin eine Komponente der ersten Phase ein polymerisierbares Monomer und die erste Behandlung ein Polymerisationsschritt zur Polymerisation des polymerisierbaren Monomers ist, wodurch die Skelettstruktur ausgebildet wird.

5. Verfahren nach Anspruch 4, worin der Polymerisationsschritt durch Erwärmen mindestens eines Initiatorvorläufers initiiert wird, der in der wässrigen Phase enthalten ist, und/oder mindestens eines Initiatorvorläufers, der in der Ölphase enthalten ist.

6. Verfahren nach Anspruch 5, worin der Polymerisationsschritt durch Erwärmen mindestens eines Initiatorvorläufers in der wässrigen Phase initiiert wird, und worin der Initiatorvorläufer Kaliumpersulfat ist.

7. Verfahren nach einem der Ansprüche 4 bis 6, worin das mindestens eine polymerisierbare Monomer ein oder mehrere Styrole, α-Methylstyrol, Chlormethylstyrol, Vinylethylbenzol, Vinyltoluol, 2-Ethylhexylacrylat, n-Butylacrylat, Isobutylacrylat, t-Butylacrylat, Hexylacrylat, n-Butylmethacrylat, Laurylmethacrylat, Isodecylmethacrylatbutadien, Isopren, Piperylen, Allen, Methylallen, Chlorallen, Vinylchlorid, Vinylfluorid und Polyfluorolefine umfasst.

8. Verfahren nach einem der Ansprüche 2 bis 7, worin die Ölphase zudem mindestens ein Vernetzermonomer umfasst.

9. Verfahren nach Anspruch 8, worin das Vernetzermonomer Divinylbenzol ist.

10. Verfahren nach einem der Ansprüche 2 bis 9, worin die Emulsion zudem ein die Emulsion mit hoher interner Phase stabilisierendes Tensid umfasst, das Sorbitanmonooleat und/oder Glycerolmonooleat umfasst.

11. Verfahren nach einem der vorausgehenden Ansprüche, worin die erste Phase zudem ein Porogen umfasst.

12. Verfahren nach einem der Ansprüche 2 bis 11, worin die wässrige Phase zudem ein wasserlösliches, quellbares Polymer umfasst.

13. Verfahren nach Anspruch 12, worin das wasserlösliche, quellbare Polymer Polyvinylalkohol ist.

14. Verfahren nach einem der Ansprüche 2 bis 13, worin die Emulsion durch Mischen der Ölphase und der wässrigen Phase in einem Mischer mit einer Scherrate von größer als 2.000 U/min hergestellt wird.

15. Verfahren nach einem der vorausgehenden Ansprüche, worin die Skelettstruktur Poren von einer mittleren Porengröße von 0,1 µm oder weniger umfasst.

16. Verfahren nach einem der vorausgehenden Ansprüche, worin die Skelettstruktur ein poröses, vernetztes Polymermaterial umfasst.

17. Tintenstrahlempfangselement mit einer porösen, vernetzten, polymeren Flüssigkeitsempfangsschicht mit einem PolyHIPE-Material, herstellbar nach einem Verfahren, wie in einem der Ansprüche 1 bis 16 definiert, worin das PolyHIPE-Material durch eine Skelettstruktur definiert ist, die durch Poren einer mittleren Porengröße von 0,1 µm oder weniger definiert ist.

18. Verwendung eines PolyHIPE-Materials in einer Tintenempfangsschicht eines Tintenstrahlempfangselements.

## Revendications

1. Procédé de préparation d'un élément récepteur pour jet d'encre comportant une couche réceptrice de liquide, le procédé comprenant les étapes indiquées dans l'ordre suivant :
générer une émulsion comportant une première phase contenant un premier fluide porteur et une seconde phase contenant un second fluide porteur, les premier et second fluides porteurs étant immiscibles ;
appliquer l'émulsion sur un support ;
mettre en oeuvre un premier traitement sur au moins un composant de la première phase pour former et/ou maintenir une ossature du au moins un composant traité de la première phase ; et
mettre en oeuvre un second traitement sur la seconde phase pour éliminer sensiblement le fluide porteur,
ce qui permet de générer une structure poreuse de grande capacité définie par l'ossature pour pouvoir absorber rapidement l'encre.

2. Procédé selon la revendication 1, dans lequel l'émulsion est une émulsion à deux phases comprenant une première phase qui est une phase huileuse et une seconde phase qui est une phase aqueuse.

3. Procédé selon l'une ou l'autre des revendications précédentes, dans lequel l'émulsion est une émulsion à phase interne élevée.

4. Procédé selon l'une quelconque des revendications précédentes, dans lequel un composant de la première phase est un monomère polymérisable et le premier traitement est une étape de polymérisation permettant de polymériser le monomère polymérisable, ce qui permet de former l'ossature.

5. Procédé selon la revendication 4, dans lequel l'étape de polymérisation est initiée en chauffant au moins un précurseur initiateur contenu dans la phase aqueuse et/ou au moins un précurseur initiateur contenu dans la phase huileuse.

6. Procédé selon la revendication 5, dans lequel l'étape de polymérisation est initiée en chauffant au moins un précurseur initiateur dans la phase aqueuse et où le précurseur initiateur est le persulfate de potassium.

7. Procédé selon l'une quelconque des revendications 4 à 6, dans lequel au moins un monomère polymérisable contient un ou plusieurs composés choisis parmi le styrène, l'α-méthylstyrène, le chlorométhylstyrène, le vinyléthylbenzène, le vinyltoluène, l'acrylate de 2-éthyl-hexyle, l'acrylate de n-butyle, l'acrylate d'isobutyle, l'acrylate de t-butyle, l'acrylate d'hexyle, le méthacrylate de n-butyle, le méthacrylate de lauryle, le méthacrylate d'isodécyle, le butadiène, l'isoprène, le pipérylène, l'allène, le méthyl allène, le chloroallène, le chlorure de vinyle, le fluorure de vinyle et les polyfluorooléfines.

8. Procédé selon l'une quelconque des revendications 2 à 7, dans lequel la phase huileuse comprend en outre au moins un monomère de réticulation.

9. Procédé selon la revendication 8, dans lequel le monomère de réticulation est le divinylbenzène.

10. Procédé selon l'une quelconque des revendications 2 à 9, dans lequel l'émulsion comprend en outre un agent tensioactif stabilisant l'émulsion à phase interne élevée qui contient du monooléate de sorbitan et/ou du monooléate de glycérol.

11. Procédé selon l'une quelconque des revendications précédentes, dans lequel la première phase comprend en outre un agent porogène.

12. Procédé selon l'une quelconque des revendications 2 à 11, dans lequel la phase aqueuse contient en outre un polymère soluble dans l'eau pouvant gonfler.

13. Procédé selon la revendication 12, dans lequel le polymère soluble dans l'eau pouvant gonfler est l'alcool polyvinylique.

14. Procédé selon l'une quelconque des revendications 2 à 13, dans lequel l'émulsion est générée en mélangeant la phase huileuse et la phase aqueuse dans un mélangeur à une vitesse de cisaillement supérieure à 2000 tpm.

15. Procédé selon l'une quelconque des revendications précédentes, dans lequel l'ossature comprend des pores d'une taille moyenne de pore inférieure ou égale à 0,1 µm.

16. Procédé selon l'une quelconque des revendications précédentes, dans lequel l'ossature contient un matériau polymère réticulé poreux.

17. Elément récepteur pour jet d'encre comprenant une couche réceptrice de liquide polymère réticulée poreuse contenant un matériau polyHIPE, pouvant être obtenu par le procédé défini dans l'une quelconque des revendications 1 à 6, dans lequel le matériau polyHIPE est défini par une ossature comprenant des pores d'une taille moyenne de pore inférieure ou égale à 0,1 µm.

18. Utilisation d'un matériau polyHIPE dans une couche réceptrice d'encre d'un élément récepteur pour jet d'encre.
